

## UNITED STATES PATENT OFFICE

2,450,222

## SHEAR-RESISTANT GREASES

Harry V. Ashburn, Glenham, Robert S. Barnett,  
Beacon, and Oney P. Puryear, Fishkill, N. Y.,  
assignors to The Texas Company, New York,  
N. Y., a corporation of Delaware

No Drawing. Application September 7, 1945,  
Serial No. 615,074

8 Claims. (Cl. 252—42.1)

1

This invention relates to improved lubricating grease compositions and particularly to texture-stable lithium base grease compositions in which a synthetic oleaginous compound comprises part or all of the oil component.

This is a continuation-in-part of our copending application Serial No. 611,908, filed August 21, 1945.

Recent developments in the production of lubricating greases and particularly those designed for specialty equipment employing sealed bearings and operating over wide temperature ranges, have led to the use of a number of organic chemical compounds as substitutes for the conventional mineral lubricating oils. These oleaginous compounds offer a marked advantage over the mineral oils in that they possess a comparatively uniform viscosity over a wide temperature range and are not as susceptible to evaporation loss as a comparable viscosity mineral oil. These features are particularly desirable and have been used to advantage in the production of greases used in sealed life-time bearing installations and low temperature greases used in aircraft controls and the like. However, one undesirable characteristic of these so-called synthetic greases is their lack of resistance to shear. Under conditions of operation where high shearing stresses are involved, such as in ball and roller-bearing lubrication, the structure of these greases gradually breaks down and their consistency falls off until they become liquid or semi-liquid. At this point the greases no longer adhere to the lubricating surfaces and bearing failures result.

In accordance with the present invention it has been found possible to produce a lithium base synthetic grease composition which possesses not only the desirable characteristics imparted by the oleaginous compounds, but is also resistant to shear. The synthetic greases previously proposed and accepted by the industry have been prepared from the lithium soaps of the conventional fatty acid sources, such as stearic acid and other soap-forming fatty acids or their glycerides. It has been discovered that the acid component of the lithium soap is an important factor in the production of synthetic greases and that synthetic greases produced from lithium soaps of soap-forming hydroxy fatty acids or their glycerides possess exceptional texture-stability and maintain their structure with little change in consistency even after extensive working at either high or low temperatures.

This unusual characteristic of the lithium soaps of hydroxy fatty acids is applicable to those

grease compositions in which a synthetic oleaginous compound comprises part or all of the oil component. The term "synthetic oleaginous compound" as used herein embraces those organic compounds or mixtures thereof which possess lubricating qualities and may be substituted in whole or in part for the conventional mineral lubricating oils. The choice of the particular compounds used in the preparation of the synthetic grease depends upon the type of lubrication and the temperature range within which the grease is intended to be operated. In general, these compounds are adapted to specialized lubrication outside the conventional lubricating temperature ranges, such as ultra-low temperature operation found in refrigeration systems and arctic service lubrication, or to general purpose lubrication over a wide lubricating temperature range which was previously unattainable through the use of a single mineral lubricating oil due to their high viscosity change over such wide temperature ranges.

As a general proposition, certain factors are prerequisite in the compounds falling within the category of synthetic oleaginous compounds. These compounds are necessarily chemically and physically stable liquids at the temperatures of operation and possess a minimum viscosity of 0.5 centistoke within the lubricating temperature range. Furthermore, the vapor pressure of these compounds in the lubricating temperature range is substantially negligible, although under conditions of flooded lubrication, where evaporation loss is not too critical, compounds of measurable vapor pressure may be used.

Inasmuch as the primary requisites of the oleaginous compounds are physical in nature, they cannot be conclusively defined in terms of their chemical structure. However, the majority of these compounds are polar compounds with oxygen as the principal type of polar constituent. Another general observation is that, in the compounds of a given chemical classification, those of comparatively high molecular weight possess the least change in viscosity per change in temperature. The types of compounds which are recognized or have been proposed as synthetic oleaginous compounds include the aliphatic ethers, aromatic acid esters, aliphatic mono- and di-carboxylic acid esters, phosphorus acid esters, and halogenated aromatic compounds. For the purposes of the present invention and as illustrative of the synthetic oleaginous compounds contemplated by the invention, those compounds falling within the category of aliphatic dicar-

boxylic acid esters are preferred. The compounds within this particular class are the esters of such acids as sebacic, adipic, pimelic, azelaic, alkenylsuccinic, alkylmaleic, etc. The esters thereof are preferably the aliphatic esters and particularly the branched chain aliphatic esters. Specific examples of the preferred oleaginous compounds are di-2-ethylhexyl sebacate, di-sec-amyl sebacate, di-2-ethylhexyl alkenylsuccinate, di-2-ethoxyethyl sebacate, di-2-(2'-methoxyethoxy) ethyl sebacate, di-2-(2'-ethylbutoxy) ethyl sebacate, di-2-butoxethyl azelate, di-2-(2'-butoxyethoxy) ethyl alkenylsuccinate, triethylidene sorbitol, di-2-butoxyethyl alkenylsuccinate, etc.

These oleaginous compounds may be used as the sole oil component of the greases or they may be blended with a mineral lubricating oil as desired. In some instances where the soap component is to be formed in situ it is desirable to conduct the saponification in the presence of mineral oil which is inert to the reaction and then add the oleaginous compound. This would result in the combination of mineral oil and oleaginous compound as the oil component of the finished grease. Furthermore, various addition agents may be incorporated with the oleaginous compounds to impart other desirable characteristics. Thus, an extreme pressure agent may be incorporated to improve the anti-wear characteristics of the compound or an anti-oxidant may be incorporated to improve the anti-oxidant properties of the compound and/or the finished grease.

The lithium soaps which have been found to contribute to the desirable attributes of the synthetic greases are those in which a soap-forming hydroxy fatty acid constitutes at least part of the acid component. The soap-forming hydroxy fatty acids contemplated herein are those containing at least 12 carbon atoms in the molecule and one or more hydroxyl groups, as well as mixtures thereof. These hydroxy fatty acids may be obtained from natural sources, such as castor oil, or may be prepared by the classical synthetic methods, such as oxidation of unsaturated fatty acids or catalytic oxidation of petroleum oils and waxes with extraction and fractionation to the desired molecular range. In the practice of the invention, as described herein, 12-hydroxy stearic acid and hydrogenated castor oil will be used as the representative types of hydroxy fatty acids and their glycerides. These acids are preferred because of their advantage of availability and cost which renders them competitive to the conventional fats and fatty acids.

The soap-forming hydroxy fatty acids may be used as the sole acidic component of the lithium soaps or they may be blended or combined with the conventional fats or fatty acids in such proportions that at least 50% of the total acidic component is comprised of the hydroxy fatty acids. The choice of fats or fatty acids and the specific proportion thereof which may be blended or combined with the hydroxy fatty acids depends upon the particular metallic constituent and the type of service for which the synthetic grease is intended. In general, any of the recognized fatty acid materials normally used in grease manufacture may be used providing they are essentially saturated in character. These fats and fatty acids include mixtures of fatty acid glycerides found in naturally-occurring fats and oils, together with fractionated components thereof. The fatty acids may be a mixture of acids split off from these fats or prepared from hydrogena-

tion of fish oils, etc., or the individual acids themselves.

The choice of the particular methods of manufacture applicable to the production of the synthetic greases of the invention will depend upon the type of oleaginous compound used and whether or not mineral oil is to be used as part of the oil component. The conventional method of preparing synthetic greases is the gelling method in which the preformed lithium soap and the oleaginous compound are heated to a homogeneous solution and rapidly cooled to form the grease gel. This method of preparation possesses certain disadvantages in that it requires a preformed lithium soap which in and of itself raises the cost of the grease because of the separate saponification step required and extensive milling equipment to work the grease gel to a homogeneous consistency. However, in preparing the greases of the invention other methods of manufacture, conventional to the grease industry, may be used. A particular advantage in the use of lithium soaps of hydroxy fatty acids is the fact that the high temperatures required by the conventional gelling methods may be avoided and the preparation conducted at temperatures around 300° F. or at least those attained in a steam-heated kettle and the finished grease drawn from the kettle without requiring homogenization. Furthermore, saponification in situ is possible either in the presence of mineral oil or a synthetic oleaginous compound which is inert to the saponification reaction.

The following examples are presented as illustrating the preparation of representative synthetic greases falling within the scope of the present invention. It is to be understood, however, that these examples are merely illustrative and not definitive of the invention and as such may be modified within the scope of the invention as previously defined in accordance with the skill of the art.

#### Example I

A steam-heated kettle equipped with stirring mechanism was charged with 16.8 pounds of 10.4% lithium hydroxide solution and 9.0 pounds of water. Stirring was started at 35 R. P. M. and the lithium hydroxide solution heated to 180° F. 16.2 pounds of hydrogenated castor oil (titer—74.6° C., Sap. No.—183, hydroxyl value—165) and 22.6 pounds of a mildly refined mineral oil were then added. The kettle contents were held at 170-190° F. for four hours and 5.52 pounds of triple-pressed stearic acid were added. The temperature was then maintained at 186-190° F. for an additional hour and the kettle shut down over night. After standing over night stirring at 35 R. P. M. was begun and the saponification mixture dehydrated at 290-312° F. for four hours. At this point the soap had a very light tan color. The heat was then reduced and 12.2 pounds of mineral oil were added. The physical tests on the mineral oil and synthetic oleaginous compound are as follows:

|                                        | Mineral Oil | Di-2-Ethylhexyl Sebacate |
|----------------------------------------|-------------|--------------------------|
| Flash, COC °F.....                     | 300         | 418                      |
| Fire, COC °F.....                      | 325         | 500                      |
| Viscosity Kinematic at 100° F. cs..... | 7.73        | 12.26, 12.74             |
| Viscosity Kinematic at 210° F. cs..... | 2.08        | 3.24, 3.30               |
| Viscosity Index.....                   | 63          | 153, 155                 |

At 236° F. 160 grams of triple-pressed stearic acid were added to render the grease slightly acidic. 26 pounds of di-2-ethylhexyl sebacate

were then added slowly. At approximately 190° F. 36.60 pounds of additional di-2-ethylhexyl sebacate were added and during the addition of the ester 196.3 grams of phenyl alpha naphthylamine were added simultaneously. At this point the grease contained approximately 15% soap and possessed an A. S. T. M. penetration at 77° F. of 301-303 unworked and 317-324 worked. 5 pounds of a blend of 28% mineral oil and 72% sebacate ester and 23 grams of phenyl alpha naphthylamine were then added. The grease was finally drawn at a temperature of 166° F. and pumped through three 60 mesh screens. The product was a light cream-colored buttery grease having the following calculated composition:

|                                                           | Per cent |
|-----------------------------------------------------------|----------|
| Lithium soap (75% hydroxy stearic acid, 25% stearic acid) | 13.6     |
| Glycerine                                                 | 1.0      |
| Mineral oil                                               | 23.8     |
| Di-2-ethylhexyl sebacate                                  | 60.9     |
| Phenyl alpha naphthylamine                                | 0.5      |
| Free fatty acid                                           | 0.2      |

The foregoing synthetic grease was subjected to a dynamic shear test which was conducted in an apparatus consisting of a perforated piston reciprocating within a closed cylinder maintained at a constant temperature. In the test the grease was charged to the cylinder at a temperature of 225° F., and the piston then reciprocated at 49 strokes per minute for a period of eight hours. At the conclusion of the run the grease was removed and miniature penetrations taken. These miniature penetrations were then compared with the miniature penetrations of the grease taken before the test to determine the effect of the shearing action on the grease structure. The results obtained on the subject grease showed an original miniature penetration of 89 and a final miniature penetration of 113.

#### Example II

A grease base consisting of the lithium soaps of the combination of 75% hydrogenated castor oil and 25% triple-pressed stearic acid and mineral oil was prepared in accordance with the procedure of Example I. This grease base possessed the following calculated composition:

|              | Per cent |
|--------------|----------|
| Lithium soap | 47.2     |
| Glycerine    | 3.5      |
| Mineral oil  | 49.3     |

750 grams of the grease base were charged to a kettle and heated with stirring at 234° F. The heat was then reduced and 1020 grams of a dimethyl silicone polymer possessing a flash point above 600° F., with a kinematic viscosity of 82 cs. at 100° F. and 32 cs. at 210° F. were slowly added over a period of six and one-half hours. At this point the temperature was 147° F. and the A. S. T. M. control penetration at 77 was 203-210 unworked and 221-223 worked. 1000 grams of additional dimethyl silicone polymer were then added slowly until a control worked penetration of 345 at 78° F. was obtained. The batch was then drawn at a temperature of 176° F. The product was a smooth, light-colored, buttery grease having the following calculated composition:

|                           | Per cent |
|---------------------------|----------|
| Lithium soap              | 12.8     |
| Glycerine                 | 0.9      |
| Mineral oil               | 13.4     |
| Dimethyl silicone polymer | 72.9     |

The subject grease was tested in a so-called

grease-breakdown machine wherein a No. 204 anti-friction bearing was packed with the grease and mounted on a motor-driven shaft operating at 3450 R. P. M. and surrounded by a heating jacket. The test was started at room temperature and the bearing gradually heated, while running at a constant speed, until the temperature reached 300° F. During the period of the test the lubricating performance was noted. At the conclusion of the test the grease was removed from the bearing and examined as to change in texture and consistency. The results obtained on the subject grease indicated excellent lubrication, with no appreciable change in texture or consistency of the grease at the conclusion of the test.

In comparison therewith a commercial dimethyl silicone grease was also tested and, although supplying excellent lubrication, the grease became semi-fluid toward the end of the test and drained from the bearing when the test was stopped.

#### Example III

100 grams of lithium 12-hydroxy stearate and 25 900 grams of di-2-ethylhexyl sebacate were mixed and heated with stirring. At 350° F. the soap began to dissolve in the ester and at 390° F. was completely in solution. The solution was heated to 400° F. and poured in a thin layer on the bottom of a grease pan, taking care that no thick spots were formed. After cooling, a smooth, buttery gel was formed which showed no signs of separation. The A. S. T. M. control worked penetration of the grease gel was 240 at 77° F. The product possessed the following calculated composition:

|                             | Per cent |
|-----------------------------|----------|
| Lithium 12-hydroxy stearate | 10       |
| Di-2-ethylhexyl sebacate    | 90       |

40 This grease was tested in the dynamic shear test described in Example I in comparison with a 10% lithium stearate grease containing di-2-ethylhexyl sebacate as the sole oil component and the results obtained are as follows:

|          | Miniature Penetration | Lithium Hydroxy Stearate | Lithium Stearate |
|----------|-----------------------|--------------------------|------------------|
| Original | 126, 130              | 181.                     |                  |
| Final    | 268, 270              | Semi-fluid.              |                  |

55 Where the said application Serial No. 611,903 discloses and claims a lubricating grease composition of the synthetic ester type of lubricating base, together with a metal soap of hydroxy fatty acids or hydroxy fatty acid glycerides, and specifically a sodium soap grease of this type, the present application is restricted to a lithium soap 60 grease of this general type.

Obviously many modifications and variations of the invention, as hereinbefore set forth, may be made without departing from the spirit and scope thereof and, therefore, only such limitations should be imposed as are indicated in the appended claims.

What we claim is:

65 1. A lubricating grease composition comprising as the essential and at least major proportion of the lubricating base an oil-soluble high molecular weight high-boiling liquid aliphatic dicarboxylic acid ester within the lubricating viscosity range and possessing lubricating properties, and sufficient lithium soap of soap-forming fatty material 70 to thicken said lubricant base, said soap-forming

fatty material consisting of more than 50% by weight of a hydroxy soap-forming fatty material selected from the group consisting of hydroxy fatty acids and hydroxy fatty acid glycerides, said grease composition being texture-stable under high shearing stress.

2. A lubricating grease composition according to claim 1, wherein the said ester is a branched chain aliphatic diester of an aliphatic dicarboxylic acid.

3. A grease composition according to claim 2, wherein the said ester is a branched chain aliphatic sebacate.

4. A lubricating grease composition according to claim 3, wherein the said diester is di-2-ethyl 15 hexyl sebacate.

5. A lubricating grease composition comprising as the major portion of the composition a lubricant base consisting of a minor proportion of mineral lubricating oil and a major proportion of an oil-soluble high molecular weight high boiling liquid branched chain aliphatic diester of an aliphatic dicarboxylic acid, sufficient lithium soap of a soap-forming fatty material consisting of a major proportion of hydrogenated castor oil and a minor proportion of a saturated soap-forming fatty acid to thicken said lubricant base, glycerine resulting from the saponification of said hydrogenated castor oil, and a small proportion of an oxidation inhibitor, said grease composition being texture-stable under high shearing stress.

6. A lubricating grease composition according to claim 5, wherein said diester is di-2-ethyl hexyl sebacate.

7. A lubricating grease composition comprising 35 as the major portion of the composition a lubricant base consisting of a minor proportion of mineral lubricating oil and a major proportion of

an oil-soluble high molecular weight high boiling liquid branched chain aliphatic diester of an aliphatic dicarboxylic acid, sufficient lithium soap of about a 3:1 mixture by weight of hydrogenated castor oil and stearic acid to thicken said lubricant base, glycerine, and a small proportion of an oxidation inhibitor.

5 8. A lubricating grease composition according to claim 7, wherein the said diester is di-2-ethyl hexyl sebacate, and the said oxidation inhibitor is phenyl alpha naphthylamine.

HARRY V. ASHBURN.  
ROBERT S. BARNETT.  
ONEY P. PURYEAR.

#### REFERENCES CITED

The following references are of record in the file of this patent:

#### UNITED STATES PATENTS

| Number       | Name                | Date          |
|--------------|---------------------|---------------|
| 1,993,738    | Graves et al. ----- | Mar. 12, 1935 |
| 2,049,072    | Mikeska -----       | July 28, 1936 |
| 2,104,408    | Wiezevich -----     | Jan. 4, 1938  |
| 25 2,303,256 | Camelford -----     | Nov. 24, 1942 |
| 2,334,274    | Meadows -----       | Nov. 16, 1943 |
| 2,351,384    | Woods et al. -----  | June 13, 1944 |
| 2,376,312    | Morgan -----        | May 15, 1945  |
| 2,379,850    | Morgan -----        | July 3, 1945  |
| 30 2,380,960 | Fraser -----        | Aug. 7, 1945  |
| 2,383,147    | Morgan -----        | Aug. 21, 1945 |
| 2,390,450    | Morgan -----        | Dec. 4, 1945  |
| 2,397,956    | Fraser -----        | Apr. 9, 1946  |

#### FOREIGN PATENTS

| Number  | Country             | Date          |
|---------|---------------------|---------------|
| 406,136 | Great Britain ----- | Feb. 22, 1934 |
| 157,953 | Switzerland -----   | Jan. 2, 1933  |